

Nov. 26, 1929.

M. KLEIFOTH

1,737,285

LAMINATED FIBROUS SHEET

Filed Oct. 25, 1928

Fig. 1.



Fig. 3.



Fig. 4.



Fig. 2.



Fig. 5.



Fig. 6.



Fig. 7.



INVENTOR  
Max Kliefoth

BY

Pennie, Davis, Marin & Edmund  
ATTORNEYS

## UNITED STATES PATENT OFFICE

MAX KLEEFOTH, OF MADISON, WISCONSIN, ASSIGNOR TO C. F. BURGESS LABORATORIES, INC., OF MADISON, WISCONSIN, A CORPORATION OF DELAWARE

## LAMINATED FIBROUS SHEET

Application filed October 25, 1928. Serial No. 314,911.

My invention relates to fibrous sheets made by laying down a succession of overlapping folds of moist pulp webs and pressing the overlapping folds into a coherent sheet, as described in the application of Howard F. Weiss, Serial No. 139,476, filed October 4th, 1926. The present invention consists in an improvement in the method described in that application whereby the pulp web is divided into a plurality of narrow webs which are laid down together in contacting, side-by-side relation to form a plurality of series of overlapping folds, the folds of the different series, when compressed, interlocking with each other to form a single coherent sheet.

It is an object of my invention to provide a multi-ply paper sheet which is uniform in thickness and density and in which wrinkling of the constituent pulp folds is reduced to a minimum.

It is a further object of the invention to provide a satisfactory thin multi-ply paper sheet.

It is a still further object of the invention to provide a multi-ply paper sheet which requires a minimum of trimming at the edges.

Other objects and advantages will become clear from the following description of my improved process and from the accompanying drawings wherein:

Fig. 1 is a diagrammatic plan view of the apparatus used to make my improved fibrous sheet;

Fig. 2 is a vertical view on line 2—2 of Fig. 1;

Fig. 3 is a plan view of a portion of a sheet produced by the apparatus of Figs. 1 and 2 when a wide web is used;

Fig. 4 is a plan view of a portion of a similar sheet when the wide web is divided into a plurality of narrow webs;

Fig. 5 is a view of a single fold of pulp web, showing the distortion to which the pulp is subjected when it is laid down upon a moving conveyor;

Fig. 6 is a view of a single fold of pulp showing the wrinkles resulting from distortion; and,

Fig. 7 is a view illustrating the decreased

distortion resulting from lengthwise division of the fold.

The method of making my improved product can best be understood by referring to the accompanying drawings in which like numerals indicate like parts in the several figures.

The vat 1 of a wet machine contains the slurry of water and pulp. The usual perforate cylinder mould 2 picks up a web of pulp which is then carried to couch roll 3 around which felt 4 travels in the indicated direction. The wet pulp web is picked up and carried along on felt 4 and is then pressed by press roll 5. The moist pulp web is picked up by press roll 5 and is removed therefrom by doctor 6. This pulp web may be creped by the doctor or may be kept smooth, as desired. The pulp web 8 is then carried forward by conveyor belt 7 which is part of a hinged reciprocating looping device which is shown in another position by the dotted lines of Fig. 2. The off-take roll 9 of the hinged looping device works along a guide 10 and distributes the pulp web 8 transversely upon conveyor 11 as shown.

Tightener roll 12 functions to keep conveyor belt 7 taut and directs the return travel of belt 7 along a path which is at all times as nearly as possible of the same length as the forward path. The pulp web 8 is deposited transversely upon the conveyor 11 in a succession of overlapping folds, adjacent individual folds being spaced from each other in the direction in which conveyor 1 travels. The non-folded side edges of adjacent individual fold sections are at an angle to each other as illustrated by Fig. 3. Conveyor 11 carries the succession of overlapping folds through a continuous press 13, which may be in the form of press rolls. This operation compresses the loosely piled overlapping folds into a coherent sheet. The sheet may continue through drier 14, side trimmer 15 and cutter 16.

For economical operation, the character of the moist pulp web, as it leaves the wet machine, is fixed within fairly narrow limits. The property, known as freeness, of the pulp fibres determines the speed at which water

will pass through the screen of cylinder mould 2 and leave a web behind and also determines how thick a mat of pulp will gather before further passage of water is effectually stopped. The thickness of the pulp web and the rate at which it is formed are, therefore, quite definitely fixed and the most economical method of increasing output is to increase the width of the web.

In the formation of a single fold section, conveyor belt 7 may be considered as laying down a rectangle 17 of moist pulp web, as illustrated in Fig. 5. The movement of conveyor 11, however, distorts the shape of rectangle 17 into that of a rhomboid 18. The result is that one diagonal dimension,  $ad$ , is increased to  $ad'$ , while the other diagonal,  $bc$ , is decreased to  $bc'$ . The pulp is stretched along the longer diagonal and there is an excess along the shorter diagonal. The result is that wrinkles are formed parallel to the longer diagonal, as illustrated in Fig. 6. Furthermore, a twist is given the web at the folded edge which results in further wrinkles and a folded edge which is not straight and which requires subsequent trimming. As the speed of conveyor 11 increases each successive fold is laid down at a greater angle to the one preceding it. In a very thin sheet, for instance, one which has the thickness of only two webs, conveyor 11 travels very fast and distortion and the wrinkling effect is greatly augmented. Furthermore, it is in the thin sheets that the wrinkling effects are most noticeable and objectionable. The sheet may be subsequently pressed to a uniform thickness but the density is not uniform and the effect remains in the presence of dark veins and the appearance of "wildness."

I have found that if the wide web is divided into a plurality of narrow webs, the folds are laid down smoothly, wrinkles are absent, and the folded edges are straight and follow the side edges of the sheet closely, making less trimming necessary. Fig. 7 illustrates the fold shown in Fig. 5 after it has been cut in half lengthwise. In this case the distortion of the rectangle into a rhomboid results in dimensional changes in the diagonals of approximately only one half the magnitude of the changes resulting when a wide web is used. Further division of the web results in greater decrease in dimensional distortion and resulting strain and wrinkles. No set rule for maximum allowable width of web can be laid down. The speed of the conveyor 11, the speed of belt 7, the thickness of the pulp web, are all factors which affect the maximum allowable width. If the web has been creped it possesses more elasticity and adjusts itself more readily under distortion and the maximum allowable width is greater. In specific operations where a web several feet wide was used, it was found un-

necessary to divide it into sections less than eight inches wide.

Division of the web into a plurality of narrow webs may be accomplished by a number of means. A very narrow circular strip of paint may be applied to the cylinder mould screen to fill the meshes and prevent the passage of water therethrough. A narrow strip of tape or other extremely thin impervious material may be secured to the cylinder mould, as by gluing. The cylinder mould may be made in sections. The wide web may be cut into strips or ribbons after it is formed by causing it to come into contact with a suitable cutting edge such as a sharp edged disc, pressing against and traveling at the same speed as press roll 5. As the specific means for dividing the web forms no part of my invention, and as numerous devices well known to those skilled in the art may be employed for this purpose, I have not illustrated such means in the drawings.

Throughout the claims the term "folds" is used to define, not only the folded edge, but the entire overlapping portions formed by each reciprocation of the looping device, and the term "edge" when used in conjunction with "folds" is intended to mean either the folded edge or loop, or the nonfolded side edge of the portion of the web forming the folds.

I claim:

1. The step in the method of making a fibrous sheet of uniform thickness which comprises laying down a plurality of narrow moist pulp webs simultaneously in contacting side-by-side relation transversely upon a moving conveyor to form a plurality of overlapping folds of pulp webs.

2. The steps in the method of making a fibrous sheet of uniform thickness which comprise creping a plurality of narrow moist pulp webs, laying said creped webs in adjacent side-by-side relation transversely upon a moving conveyor to form a plurality of overlapping folds of pulp webs.

3. The method of making a fibrous sheet of uniform thickness which comprises laying down a plurality of narrow moist pulp webs in contacting side-by-side relation transversely upon a moving conveyor to form a plurality of overlapping folds of pulp webs and pressing said folds into a coherent sheet.

4. The method of making a fibrous sheet of uniform thickness which comprises laying down a plurality of narrow, moist pulp webs in contacting side-by-side relation transversely upon a moving conveyor to form a plurality of overlapping folds of pulp web, pressing said folds into a coherent sheet, and drying said pressed sheet.

5. The method of making a fibrous sheet of uniform thickness which comprises forming a suspension of pulp, forming a plurality of narrow webs from said pulp in contacting

side-by-side relation, laying down said webs together transversely upon a moving conveyor to form a plurality of overlapping folds of pulp webs, and pressing said folds into a coherent sheet.

6. The method of making a fibrous sheet of uniform thickness which comprises dividing a moist pulp web into a plurality of narrow webs, laying down said narrow webs together transversely upon a moving conveyor in contacting, side-by-side relation to form a plurality of overlapping folds, and pressing said folds into a coherent sheet.

7. As an article of manufacture, a fibrous sheet comprising a plurality of overlapping folds of a plurality of narrow pulp webs in contacting side-by-side relation, said folds having edges extending in transverse relation to the machine direction of the sheet, said edges being spaced from each other in the machine direction of the finished sheet.

8. As an article of manufacture, a fibrous sheet comprising a plurality of overlapping folds of a plurality of narrow creped pulp webs in side-by-side relation, said folds having edges extending in transverse relation to the machine direction of the sheet, said edges being spaced from each other in the machine direction of the finished sheet.

30 In testimony whereof I affix my signature.  
MAX KLIEFOTH.

35

40

45

50

55

60

65